

## UNITED STATES PATENT OFFICE

2,107,064

## PROCESS FOR SOLVENT DEWAXING OILS

Hendrikus van der Waerden, The Hague, Netherlands, assignor to Shell Development Company, San Francisco, Calif., a corporation of Delaware

No Drawing. Application April 8, 1935, Serial No. 15,290. In the Netherlands April 25, 1934

10 Claims. (Cl. 196—18)

This invention relates to a process for separating waxy substances from mineral oils, such as petroleum oils, tar oils, shale oils, brown coal distillation oils, and the like. More particularly, 5 this invention is concerned with the use of a new solvent or diluent mixture for aiding the separation of waxy substances from the oil.

Mineral oils naturally contain varying amounts of high melting hydrocarbons hereinafter, for 10 convenience, designated as "waxes" which at normal or at elevated temperatures are liquid or dissolved in the liquid hydrocarbons, but which solidify into amorphous or into crystalline form at lower temperatures. When these wax-bearing 15 oils are used at such lower temperatures the waxes may resist or obstruct the desired flow of the oil. Moreover, when the wax content is too low to impede materially the flow of oil, it may, nevertheless, cause an undesirable cloudiness. It 20 is, therefore, often necessary to effect the removal of at least a portion of these waxy constituents.

The removal of wax from oil, and more particularly the removal of mineral wax from mineral oil has in the past been accomplished by 25 the dilution of the wax-bearing oil with a suitable diluent or diluent mixture, followed by chilling the solution to precipitate the wax, and the separation of the precipitated wax by some suitable means, such as filter pressing. The function 30 of the diluent was to reduce the viscosity of the chilled mixture, whereby the separation of the wax was facilitated.

It has also been proposed to aid the separation 35 of the solid wax by using diluents possessing selective solvent properties, i. e. having a high solvent power for liquid hydrocarbons, but none or only a slight solvent power for solidified wax. Acetone, ethyl alcohol, naphthas, etc., and mixtures 40 of acetone and benzol have been suggested as diluents for this purpose.

It has, in the present invention, been found 45 that particularly good results are obtained by using as a dewaxing diluent or solvent, a mixture of one or more partially hydrogenated naphthalenes which may or may not have aliphatic side chains, such as tetrahydronaphthalene and one or more liquids having selective solvent properties but low solubility for oil, such as lower symmetrical or unsymmetrical aliphatic ketones, 50 aliphatic esters, aliphatic acids, hydroxy or keto-aliphatic acids, anhydrides of aliphatic acids, aliphatic alcohols, aliphatic carbonates, etc., as well as oxy-cyclic and nitro-cyclic compounds. 55 Specific examples of selective solvents are: ace-

tone, ethyl methyl ketone, diacetone alcohol, methyl formate, methyl acetate, ethyl acetate, acetic acid, butyric acid, lactic acid, acetic anhydride, methyl carbonate, ethyl formate, butyl alcohol, quinoline, iso-quinoline, pyrrole, furfural, etc. The aliphatic solvents are characterized by having not more than five carbon atoms in the molecule. Although I have enumerated a number of solvents which may be used with hydrogenated naphthalene in a dewaxing solvent 10 mixture, my invention is not limited thereto, but may be employed in connection with other analogous solvents.

These constituents may be mixed in any desired proportion, depending upon the amount of wax to be separated, upon the dilution ratio and upon the separation temperature. It is essential that the mixture have a high solvent power for the liquid hydrocarbons and a low solvent power for the solid hydrocarbons at the temperature at which the separation of the solid from the liquid hydrocarbons occurs. The low solubility selective solvents, of which the ketones constitute the preferred group, are effective for separating solid and liquid oil components, due 25 to the difference in solubility of such oil components in these solvents, but this action is limited by their low solubility in the oil at the low or moderate temperatures of the dewaxing operation. The partially hydrogenated naphthalene increases the solubility of oily components. The optimum condition is that at the filtering 30 temperature the oil is just completely dissolved, an efficient precipitation of the wax without occlusion of oil being thus obtained. Under certain 35 conditions the partially hydrogenated naphthalene has the further effect of reducing the viscosity of the oil to aid in the separation of the liquid and solid phases. With these desiderata and the function of the components of my 40 mixture in view, the proper ratio may be readily determined empirically in each particular case. It is often preferable to use a eutectic mixture of these constituents such as a eutectic mixture of an aliphatic ketone having not more 45 than 5 carbon atoms in the molecule and a partially hydrogenated naphthalene.

Suitable mixtures may, for example, consist of 50 parts of tetrahydronaphthalene and 50 parts of acetone, or 75/25, or 25/75, according as the 50 nature of the oil is more paraffinic or more aromatic. The dilution ratio (i. e. volume ratio of oil to solvent mixture) will be determined by the viscosity wanted at the filtration temperature and will vary with the character of the oil, but 55

can be readily determined in any particular instance by those skilled in the art. By the term "effective quantity" as used in the claims, I mean the quantity of solvent mixture which will maintain sufficient oil in solution to produce its substantial separation from the wax which is precipitated, and which will produce an oil-solvent mixture of the desired viscosity.

In carrying out my invention, a wax-bearing oil may be mixed with my solvent mixture at normal or at elevated temperature, chilled to precipitate the wax, and separated from the precipitated wax, which may be either crystalline or amorphous, by any known means, such as filter 10 pressing, centrifuging, or cold settling. The separation temperature largely determines the melting point and the quantity of the wax which is separated. The dewaxing may be conducted either as a continuous or as a batch process. It 15 is sometimes desirable to precipitate the wax in several stages, thereby producing a number of waxes of different melting points. According to this method, the first precipitation and separation is carried out at a temperature which is sufficiently high to solidify only the highest melting 20 components, and the filtrate is chilled to effect further separation of wax at one or more stages at successively lower temperatures. The amount of the dewaxing mixture in the oil may, moreover, be varied at each stage so as to be present 25 in the correct quantity to dissolve substantially all of the oil at the particular temperature while not causing the dissolution of substantial amounts of the solid wax. Thus, it is often necessary to add more dewaxing solvent at each successive 30 stage.

It is generally desirable, but not essential, to produce a homogeneous oil-wax-solvent system prior to the precipitation step. To achieve this 40 condition the system is heated to a temperature below its boiling point and then chilled to precipitate the wax.

Under certain conditions, as when a moderately high pour point is permissible, and/or when, 45 in a multiple stage process, it is desired to obtain high melting wax in the first stage, the precipitation of the wax may, with my solvent mixture, be effected at temperatures which are the same as or only slightly below normal. Under these 50 conditions extreme chilling is obviated.

The solvent mixture may be recovered from the oil and from the wax by evaporation or by 55 vacuum distillation and reused. A particular advantage of the process according to this invention is that evaporation losses during the dewaxing operation and in the recovery of the dewaxing solvents are smaller for the present method than for methods employing mixtures used heretofore.

An example of the use of a diluent mixture for 60 dewaxing is as follows, it being understood that my invention is not limited to the particular substances, ratios, quantities and operating conditions appearing therein.

One part of a lubricating oil having a pour-point of 37° C. was mixed with three parts of a 65 mixture of equal quantities of acetone and tetrahydronaphthalene, chilled to -20° C. and filtered. The pour-point of the filtrate was -13° C.

It will also be understood that in some cases 70 a three-component mixture containing partially hydrogenated naphthalene, a selective solvent of low solvent power, and a third substance of intermediate solvent power, such as an ether, may be used. The additional component should, preferably, have some selective solvent properties.

Moreover, it is not necessary to mix all of the components of the solvent mixture before dissolving them in the oil. Thus, the partially hydrogenated naphthalene may be added first, either alone or with small amounts of the second component, followed by the addition of the requisite amount of the second component.

I claim as my invention:

1. A process for dewaxing oil by mixing the oil with a liquid dewaxing agent having a high solvent power for the oily components of the wax-bearing oil but low solubility for its waxy components, chilling the resulting mixture to precipitate waxy components and separating the precipitated material from the oil-containing solution, characterized by the use as the dewaxing agent of a mixture comprising a partially hydrogenated naphthalene and a selective solvent having a low solvent power for oil.

2. A process for dewaxing oil by mixing the oil with a liquid dewaxing agent having a high solvent power for the oily components of the wax-bearing oil but low solubility for its waxy components, chilling the resulting mixture to precipitate waxy components and separating the precipitated material from the oil-containing solution, characterized by the use as the dewaxing agent of a mixture comprising a partially hydrogenated naphthalene and an aliphatic ketone having not more than five carbon atoms in the 30 molecule.

3. A process for dewaxing oil by mixing the oil with a liquid dewaxing agent having a high solvent power for the oily components of the wax-bearing oil but low solubility for its waxy components, chilling the resulting mixture to precipitate waxy components and separating the precipitated material from the oil-containing solution, characterized by the use as the dewaxing agent of a mixture comprising tetrahydronaphthalene and an aliphatic ketone having not more than five carbon atoms in the molecule.

4. A process for dewaxing oil by mixing the oil with a liquid dewaxing agent having a high solvent power for the oily components of the wax-bearing oil but low solubility for its waxy components, chilling the resulting mixture to precipitate waxy components, and separating the precipitated material from the oil-containing solution, characterized by the use as the dewaxing agent of a mixture consisting of tetrahydronaphthalene and acetone.

5. A process of dewaxing mineral lubricating oils comprising the steps of mixing a wax-bearing oil with an effective quantity of an aliphatic ketone having not more than five carbon atoms in the molecule, precipitating the wax from the resulting mixture in the presence of a quantity of partially hydrogenated naphthalene, said quantity being sufficient to prevent the separation of substantial amounts of oil from the oil-solvent mixture during the precipitation, and mechanically removing the precipitated oil from the solution.

6. A process of dewaxing mineral lubricating oils comprising the steps of mixing a wax-bearing oil with an effective quantity of an aliphatic ketone having not more than five carbon atoms in the molecule, precipitating wax from the resulting mixture in the presence of tetrahydronaphthalene, said quantity being sufficient to prevent the separation of substantial amounts of oil from the oil-solvent mixture during the precipitation, and mechanically removing the precipitated oil from the solution.

7. A process of dewaxing mineral lubricating oils comprising the steps of mixing a wax-bearing oil with effective quantities of an aliphatic ketone having not more than five carbon atoms in the molecule, and a partially hydrogenated naphthalene, said quantities being sufficient to prevent the separation of substantial amounts of oil with the solidified wax when the oil-wax-solvents mixture is chilled, and chilling the resulting mixture to solidify the wax.

8. A process of dewaxing mineral lubricating oils comprising the steps of mixing a wax-bearing oil with an effective quantity of the eutectic mixture of an aliphatic ketone having not more than five carbon atoms in the molecule, and a partially hydrogenated naphthalene, said quantity being sufficient to prevent the separation of substantial amounts of oil with the solidified wax when the oil-wax-solvents mixture is chilled, and chilling the resulting mixture to solidify wax.

9. A process for dewaxing mineral lubricating oil comprising the steps of mixing a wax-bearing

oil with an effective quantity of an aliphatic ester having not more than five carbon atoms in the molecule, precipitating the wax from the resulting mixture in the presence of a quantity of partially hydrogenated naphthalene, said quantity being sufficient to prevent the separation of substantial amounts of oil from the oil-solvent mixture during the precipitation, and mechanically removing the precipitated oil from the solution.

10. A process for dewaxing mineral lubricating oil comprising the steps of mixing a wax-bearing oil with an effective quantity of an aliphatic alcohol having not more than five carbon atoms in the molecule, precipitating the wax from the resulting mixture in the presence of a quantity of partially hydrogenated naphthalene, said quantity being sufficient to prevent the separation of substantial amounts of oil from the oil-solvent mixture during the precipitation, and mechanically removing the precipitated oil from the solution.

HENDRIKUS VAN DER WAERDEN.